

# UNITED STATES PATENT OFFICE.

EMORY I. NICHOLS, OF SAN FRANCISCO, CALIFORNIA.

## COPYING-PAPER.

SPECIFICATION forming part of Letters Patent No. 359,170, dated March 8, 1887.

Application filed July 30, 1885. Serial No. 173,095. (No specimens.)

*To all whom it may concern:*

Be it known that I, EMORY I. NICHOLS, of the city and county of San Francisco, State of California, have invented an Improvement in 5 Copying-Paper; and I hereby declare the following to be a full, clear, and exact description of the same.

My invention relates to a new and useful copying-paper; and my invention consists in 10 a piece or sheet of blotting-paper saturated and coated slightly with a liquid solution of glue, water, ammonia, sugar, and glycerine.

In order that my invention may be more 15 fully understood and can be practiced by those desiring to do so, I will now describe particularly the manner of making and the manner of using the paper, together with its advantages.

I first take a sheet of any flexible and 20 absorbent material or unsized paper, such as blotting-paper. This is to form the basis of my copying-paper. I then prepare a mixture of the following ingredients, in the proportions specified: best white glue, four parts; pure 25 water, five parts; ammonia, three parts; sugar, two parts; glycerine, eight parts. This mixture I prepare in the following manner: The glue is soaked in the water and ammonia until it is soft. Heat is then applied until the glue 30 is melted, when the sugar and glycerine are added and the composition brought to a boiling-point; or treat until thoroughly mixed. This mixture is applied, while still hot, to the sheet of blotting-paper, the application being 35 made with a brush or otherwise, as may be convenient. It is laid on in sufficient quantity to cause it to penetrate or saturate the paper and leave a thin coating or film on its surface. I then let the paper so saturated and coated 40 stand two or three days, when it will be ready for use.

The manner of its use is as follows: First 45 wet the prepared paper on that surface on which the coating of composition is, the wetting being done with a common copying-brush or sponge. Keep the same wet from one to two minutes, according to the density of the lines required to be transferred. Then place the writing, drawing, or other delineation 50 (which has been made with a suitable ink, such as the aniline inks used in the hecto-

graph process) with the writing side to the prepared paper. Then press the writing on the copying-paper with the hand, or run a roller over it should the same be a drawing 55 of large size. Let it stand for about a minute, and then remove it, when it will be found that the writing or other delineation is impressed on the surface of the copying-paper. Now take the sheet upon which the impression is to 60 be transferred and place it upon the copying-paper, smoothing it over gently. When removed the impression will be upon it in the right manner. Successive sheets are thus treated.

Should the copying-paper become dry or 65 sticky, as it will after every few impressions, it should be moistened again with water. After the operation has been completed the copying-paper is laid aside, and in about twenty-four 70 hours it is ready for use again to take a fresh impression and transfer it to other paper. The operation can be repeated from time to time by simply moistening with water the surface of the copying-paper.

I am aware of the ingredients which form 75 the impression pad or surface of the hectograph, and a comparison of said ingredients with those which I use in preparing my copying-paper will show that several are common 80 in both. By an examination of the description of said hectograph it will be seen that one of the essentials is that the pad or impression-surface shall have the property of remaining moist. This property is imparted to it by the 85 large proportion of glycerine which is used in the composition. It will be seen that the proportion of glycerine in my composition with which I treat the blotting-paper is with respect to the glue as two to one, while in the 90 hectograph the proportion of glycerine to gelatine is as four to one. This results in a very essential and important difference, which I will now point out. The hectograph impression-surface remains always moist and non-absorbent, which necessitates the washing off of 95 the impression after one operation of copying has been completed. My copying-paper does not remain moist, but has, on the contrary, to be frequently wet with water; but it does not have to be washed to remove the impression, as the whole of it will be absorbed 100

by laying the sheet aside for a certain length of time. This effect I ascribe to the presence of the ammonia and the sugar in the composition with which I treat the paper. By not 5 having to wash it I save much trouble and inconvenience.

Having thus described invention, what I claim as new, and desire to secure by Letters Patent, is—

- 10 A manifold paper consisting of a piece or sheet of absorbent material saturated and

slightly coated with a solution or composition of matter consisting of glue, water, ammonia, sugar, and glycerine, prepared substantially in the proportions specified.

In witness whereof I have hereunto set my hand.

EMORY I. NICHOLS.

Witnesses:

S. H. NOURSE,  
C. D. COLE.

15